# EUROPEAN PATENT SPECIFICATION

(11) **EP 0 753 358 B1**
(45) Date of publication and mention of the grant of the patent: **12.03.2003**
(21) Application number: 96110839.6
(22) Date of filing: 04.07.1996
(51) Int. Cl.: B05D 1/00, B05D 7/02, B05D 1/04, B05D 7/00

(54) **Method of painting elements made from plastics, and elements formed thereby**
Verfahren zum Anstreichen von Kunststoffgegenstände und Gegenstände nach diesem Verfahren hergestellt
Méthode pour peindre des éléments en plastique et éléments ainsi fabriqués

(30) Priority: 07.07.1995 IT TO950574
(43) Date of publication of application: 15.01.1997
(73) Proprietor: FIAT AUTO S.p.A., 10135 Torino (IT)
(72) Inventor: Chiesi, Franco, 14017 Valfenera (IT)
(74) Representative: Plebani, Rinaldo

(56) References cited:
- EP-A- 0 693 323
- FR-A- 2 695 048
- US-I4- T 982 004

## Description

The present invention concerns an improved method of painting applicable to elements formed from synthetic plastics materials, in particular, motor-vehicle body components made from composites, which avoids the risk of bubbles and/or blisters forming in the layer/layers of paint/paints. The invention also relates to elements formed from painted plastics material, which have a high quality of surface finish and do not require, except in exceptional cases, subsequent repairs to the paintwork.

It is known in the motor vehicle industry, that vehicle body components (bonnets, doors, etc) made from synthetic plastic materials are being used increasingly and these may be formed in complex shapes and/or with low weights, both of which factors are impossible to achieve with sheet steel elements of substantially the same dimensions. Composites such as SMC, BMC, etc based on thermosetting plastics resins of the vinyl ester/polyester type are preferably used to make such components.

Once moulded, such components must be painted with the same paints and, substantially, the same production cycle as sheet-steel parts in order to ensure perfect aesthetic conformity between parts of the same motor vehicle made from different materials. To this end, a base layer of an electroconductive material is applied directly to the surfaces of the plastics elements to be painted, this base usually comprising a single-component conductive primer which polymerises at a relatively high temperature (approximately 150°C).

Typically, the primer is spread in a layer of predetermined thickness (approximately 30 microns) and the treated element is then stoved in an oven, causing polymerisation of the primer layer which hardens to form a porous, transparent, conductive film on the surface of the plastics element to be painted. By virtue of the conductivity of the primer the element may then be painted by conventional methods as if it were an element made from sheet steel; this also improves the adhesion of the layers of paint applied successively to the surface of the element. After all the paint/paints have been applied, the elements are again stoved at a high temperature (150°C) to cause the polymerisation of the paint layers.

However, during the painting process described and, in particular, during the final stage of stoving of the painted elements, problems, such as the formation of bubbles or blisters in the paint layer, frequently arise; this occurs particularly frequently in the case of vehicle body parts formed from composites based on thermosetting resins such as BMC and SMC. This problem requires the elements upon which surface bubbles have developed to be repaired manually by means of sanding to remove the layer of paint ruined by the bubble, filling and repainting: this is slow and involves a significant increase in manufacturing costs; in addition, during the subsequent stoving of the repainted part, the problem of bubbles forming in the paint layer may arise again leading, in the most serious cases, to the component being discarded.

The problems described are the reason for the lack of extensive use, in the motor vehicle industry, of vehicle body parts made from composites, which use is instead limited to small-scale production, to cover so-called "niche" productions, such as special vehicles (convertibles, single-compartment family vehicles etc).

The problem is not solved by US-I-T982004 which provides a method wherein two primers, one of which able to give raise to a gas impermeable layer, are polymerized at the same temperature.

The aim of the invention is to provide an improved method of painting elements made from synthetic plastics materials, in particular vehicle body parts made from composites, which does not have the disadvantages described, in particular being free from the risk of bubbles forming in the paint layer during the stoving stage.

On this basis, the invention therefore provides a method of painting applicable to elements made from synthetic plastics material, in particular motor vehicle parts made from composites, as claimed in claim 1. Therefore, firstly, at least one base layer of a predetermined thickness of a polymerisable electroconductive material is applied to a surface of a said element to be painted and, subsequently at least one layer of paint is applied on top of the said base layer of polymerisable material; then
- the element is brought to a first predetermined temperature to cause the polymerisation of the said base layer of polymerisable electroconductive material;
before the said base layer of polymerisable electroconductive material is applied, the method includes the following steps:
(a) - applying a continuous layer of a second polymerisable material to the said surface to be painted, the said second material being of a type which, once polymerised, can form a layer which is impervious to any gaseous substance and which is completely polymerisable by heating to a second predetermined temperature below both the said first predetermined temperature and the lowest temperature of vaporisation of the monomers forming the said synthetic plastics material constituting the said element to be painted;
(b) - heating the element, with the said surface to be painted covered with the said layer of the second polymerisable material, to the said second predetermined temperature until the said second polymerisable material is completely polymerised;
in such a way that the layer of the said polymerisable electroconductive material is deposited, not directly on the said surface to be painted, but on a gas-impermeable layer formed from the said polymerised second material which covers the said surface to be painted completely.

In particular, the said element to be painted is formed from a material based on thermosetting vinyl ester/polyester resins, and the said second polymerisable material is constituted by a catalysed two-component polyurethane transparent paint which is completely polymerisable by heating to just 60°C. The said second polymerisable material is applied to a layer formed by a polyester-based adhesion promoter which is applied directly to the surface to be painted.

The invention also relates to a painted element as claimed in Claim 8.

In this way, any risk that bubbles will form in the paint layer as a result of the final stoving to which the painted elements must be subjected to polymerise the layer/layers of paint applied is completely avoided. In fact, the Applicant has established by extensive experimentation that the formation of bubbles in the paint, a well known disadvantage which has until now greatly limited the extensive use of painted composite elements in a vehicle body, is due to the vaporisation, during stoving (which occurs at approximately 150°C), of a small proportion of the monomers, forming the resin/resins from which the element to be painted is formed which have not polymerised or are only partly polymerised and which, during the pressing, remain trapped in micropores, invisible to the naked eye, close to the surface of the element and in communication with the exterior.

However, the application of the catalysed two-component polyurethane paint layer directly to the surface to be painted (with the interposition solely of the adhesion promoter) and its polymerisation before the application of the conventional layers of primer and paint to the surface to be painted allows a gas-impermeable layer to be formed on the surface itself, forming a gas-tight seal over the surface pores which may contain unpolymerised or partially-polymerised monomers.

Consequently, when these vaporise during the final stoving of the painted element, the gases produced are no longer able to reach the painted surface and pass through the porous primer layer to penetrate the layers of paint being polymerised and so form the known bubbles. The polymerisation of the layer of gas-impermeable material at a low temperature (about 60°C), by virtue of the use of catalysed paints, also guarantees that no monomers can vaporise during the polymerisation of this sealing layer, risking localised damage in the layer which is still being polymerised, which could mean that the layer itself is not completely impermeable.

These and other characteristics of the invention will become clearer from the following description of a preferred embodiment, given by way of non-limitative example, with reference to the accompanying drawings, in which:
- Figure 1 represents schematically the mechanism by which bubbles are formed in a layer of paint applied to a surface of an element made from plastics material; and
- Figure 2 represents schematically in section the structure of a plastics element painted according to the invention.

With reference to Figures 1 and 2, the reference numeral 1 indicates an element formed from a synthetic plastics material, for example, a panel pressed from a composite material and forming a vehicle body part, for example, of a motor vehicle, such as a bonnet, a door, etc. Here and in the following description, the composites are considered, for simplicity, as a subclass of synthetic materials being, as is known, constituted by a reinforcing agent (glass, carbon, kevlar fibres, etc, regardless of how it is formed and distributed), encapsulated in a matrix constituted by one or more synthetic plastics resins obtained by the polymerisation of one or more monomers.

The panel or element 1 has a surface 2 covered by a paint coating 3 (possibly constituted by a plurality of superposed thinner layers of diverse materials); the surface 2 also contains pores 4 (only one of which is illustrated on an enlarged scale in Figure 1), at least some of which are partially filled with grains 5 of unpolymerised or only partially polymerised monomers; the grains 5 are formed from the same monomers as those used to form the resin/resins constituting the synthetic plastics base material from which (with the addition of the fillers) the element or panel 1 is made, and are the inevitable result of the known process for forming the panel or element 1 which is, for example, obtained by injection moulding, compression moulding, or injection-compression moulding.

In the present case described, which concerns elements 1 intended for motor vehicle bodies, the resin/resins forming the element or panel 1 are thermosetting vinyl ester/polyester resins as the element/panel 1 is moulded from a composite of the SMC, BMC or similar type.

As determined by the Applicant, because of the microstructure of the panel/element 1, when the painted element 1 is heated to polymerise the multi-layered coating 3, the grain 5 vaporises creating gases (shown by the arrows 6) which, together with any air which may be trapped in the pore 4, expand and leave the pore 4, causing the coating 3 to swell which, as it is in the polymerising phase, is soft and plastic, although already mostly impermeable to gases; the gases 6 are thus not able to escape and they collect above the pore 4 and below the coating 3, creating a bubble 7. It has been determined that the sizes of the bubbles 7 are an order of magnitude greater than those in the pores 4, which may vary from several microns to several millimetres: consequently, the bubbles 7 which form are between 1 and 10 millimetres in diameter or more.

This fact confirms the validity of the interpretive model described above: if, in fact, the formation of the bubbles 7 were not due primarily to the vaporisation of monomers which are not 100% polymerised within the pores 4, the size of the bubbles would in practice be limited to 5/7 of those within the pores 4 (a value corresponding to the variation in volume of the air in the pores 4 caused by thermal expansion) and, consequently, only extremely small bubbles would form. In addition, the model is further confirmed by the fact that, in current practice, bubbles also form again at exactly the same places on elements 1 that have already experienced the phenomenon and which have been repaired (by sanding, filling and repainting of the places where bubbles formed), as soon as the piece is heated again to polymerise the paint in the repaired areas.

With reference to Figure 2, the known phenomenon illustrated in Figure 1 is avoided, according to the invention, by means of a particular structuring of the multi-layered coating 3. In practice, a coating 3a is formed according to the invention on the surface 2 and, starting with the layer adjacent the surface 2, comprises two superimposed films B and A; the film A corresponds to conventional coatings, such as that in Figure 1, while the film B includes, in turn, a first continuous layer 10 applied directly to the surface 2 to cover it completely, being approximately 30 microns thick and formed from a polyester-based adhesion promoter ("Barrier"), for example, 487567 from the firm PPG Industries Inc, USA, and a second layer 11, also continuous and applied directly to the layer 10 so as to cover the surface 2 completely, being between 30 and 40 microns thick and formed from a material which polymerises at low temperature (approximately 60°C) and is impermeable to gaseous substances such that the layer 10 is completely gas-impermeable.

In the present case, the layer 11 is formed from a catalysed two-component transparent polyurethane paint, such as, for example, 228003 obtained from PPG Industries Inc. The film A, instead, is, as already stated, constituted by a conventional multi-layer coating including, in the present case: a first layer 12 of thickness which may vary between 20 and 30 microns formed from an electrically-conductive polymerisable primer of the single-component type, for example, 487538, also from PPG Industries Inc, having a stoving temperature (for polymerisation) of about 150°C; a second layer 13, approximately 40 microns thick, formed from an undercoat paint, for example, "base coat" 400085/1 from HERBERTS GmbH, WUPPERTAL (D); a third layer 14, approximately 30 microns thick, formed from enamel and defining the real paint layer; and a surface layer 15 of approximately 30 microns thick, formed from a protective transparent polymer, for example, a "lacquer" of any known type.

According to the invention, the layer 10 is first of all applied, for example, by spraying to the surface 2 of the untreated element or panel 1 to be painted and then the layer 11 of two-component paint, which is applied by a "wet on wet" technique, that is, while the underlying film of material just applied is still wet due to the, as yet, incomplete evaporation of the solvent used. The element 1, with only the layers 10 and 11 covering the surface 2 completely, is then stoved in an oven at a temperature which causes the rapid polymerisation of the material forming the layer 11; since one is dealing with a catalysed paint, the latter polymerises completely in approximately 45 minutes on heating of the element 1 to merely 60°C. At such a low temperature, which is certainly below the lowest temperature of vaporisation of any monomers in the pores 4, these latter are not able to generate any gas whereby the layer 11 polymerises completely, thereby becoming impermeable to any gaseous substance rapidly and without any damage.

Once the polymerisation of the layer 11 is complete, the element 1 is cooled and the layer 12 of conductive primer is first applied thereto in a known way followed by the layers 13, 14, 15 of paint proper; these layers, starting from the base layer 12, are not however applied directly to the surface 2, as in the prior art, but to the layer 11 which, as already said, is completely impermeable to gases when fully polymerised; instead, the layer 12, which acts as a base for the in-line application of the three layers of paint 13, 14 and 15 by the same known methods as for body parts made from sheet steel is, as is known, porous and therefore permeable to gaseous substances which are able to diffuse through it, in the direction of the thickness, as already described in Figure 1.

Therefore, when the stoving stage necessary for polymerisation of the layer 12 is reached (as well as any subsequent stoving to cause the other layers of the film A to polymerise, whether separately or together), which step is executed by bringing the element 1 to a temperature of 140-160°C (on average 150°C) for approximately 30 minutes (always to a temperature much higher than that for the polymerisation of the layer 11), the gases which arise in the pores 4 (Figure 2) as a consequence of the vaporisation of the monomers therein, leave the pores 4 to diffuse towards the film A but, before reaching the porous layer 12 which is still polymerising, encounter the gas-impermeable layer 11 which is already completely polymerised and therefore very rigid and of high mechanical strength. Consequently, the gases 6 are sealed in the pores 4, below the layer 11 and are therefore prevented from deforming the plastic layers 12-15 and creating bubbles 7. Any risk of the formation thereof is therefore avoided.

## Claims

1. A method of painting applicable to elements formed from synthetic plastics materials, in particular components of motor vehicles formed from composites, **characterized by** comprising the steps of:
- applying to a surface (2) of a said element (1) to be painted a layer (11) of a first polymerisable material, the said first polymerisable material being of a type which, once polymerised, can form a layer which is impervious to any gaseous substance and which is completely polymerisable by heating to a first predetermined temperature;
- heating the element (1), with the said surface (2) to be painted covered with the said layer of first polymerisable material, to the said first predetermined temperature until the said first polymerisable material is completely polymerised to form a gas-impermeable layer (11) which covers the said surface to be painted completely;
- applying to the said surface (2) at least a base layer (12) of a predetermined thickness of a polymerisable electroconductive material, which is polymerisable by heating to a second predetermined temperature;
- heating the element (1) to the said second predetermined temperature to cause the polymerisation of the said base layer (12) of polymerisable electroconductive material, in such a way that the said base layer (12) of polymerisable electroconductive material is deposited not directly on the said surface (2) to be painted, but onto the said gas-impermeable layer (11);
- applying at least one layer of paint (13, 14) on top of the said base layer (12) of electroconductive polymerisable material;
the said first polymerisable material being selected in such a way that the said first predetermined temperature is below both the said second predetermined temperature and the lowest temperature of vaporisation of the monomers forming the said synthetic plastics material constituting the said element to be painted.

2. A method according to Claim 1 in which the said element (1) to be painted is formed from a material based on thermosetting vinyl ester/polyester resins, **characterised in that** the said second polymerisable material is constituted by a catalysed two-component polyurethane transparent paint.

3. A method according to Claim 2, **characterised in that** the said first polymerisable material is applied on top of the said surface (2) to be painted to form thereon a layer (11) of between 30 and 40 microns thick.

4. A method according to Claim 2 or Claim 3, **characterised in that** a layer (10) of adhesion promoter for the said first polymerisable material is applied in direct contact with the said surface (2) to be painted; this first polymerisable material being applied immediately on top of the said layer (10) formed from the adhesion promoter.

5. A method according to Claim 4, **characterised in that** a polyester-based adhesion promoter ("Barrier") is used, applied to the said surface (2) to be painted in a continuous layer (10) at least 30 microns thick; and **in that** the said catalysed two-component polyurethane paint is chosen such that it is completely polymerised at a temperature of 60°C.

6. A method according to Claim 5, **characterised in that** the said second two-component polyurethane paint is delivered to the said surface (2) by a "wet on wet" technique.

7. A method according to any one of Claims 2 to 6, **characterised in that** the said electroconductive polymerisable material is a single-component primer which is polymerisable by heating to a temperature of at least 140-150°C.

8. A painted element (1) formed from a synthetic plastics material, in particular a vehicle body part formed from a composite material, comprising a panel (1) pressed from at least one synthetic plastics resin, at least one visible surface (2) of which is covered by a plurality of layers of polymerisable materials including at least one layer of paint (13, 14); the said plurality of layers of polymerisable materials comprising, in order starting with the layer adjacent the said surface (2), a first, gas-impermeable layer (11), and a second, gas-permeable layer (12), both formed from respective different polymerised materials; the material forming the first layer (11) having a chemical composition such that it polymerises completely on heating to a first predetermined temperature; the material forming the second layer (12) having a chemical composition such that it forms an electroconductive primer for receiving the said at least one layer of paint (13, 14), and which polymerises on heating to a second predetermined temperature which is substantially equal to that needed to polymerise the at least one layer of paint;
the element being **characterised in that** the material forming the first layer (11) has been selected in such a way that said first predetermined temperature is below both the said second predetermined temperature and the lowest temperature of vaporisation of the monomers forming the said synthetic plastics resin from which the said panel is formed.

9. A painted element according to Claim 8, **characterised in that** the said panel (1) is formed from at least one thermosetting vinyl ester/polyester-based resin; and **in that** the first layer (11) is formed from a two-component polyurethane paint; the said first layer (11) being between 30 and 40 microns thick and being applied over a layer (10) of a material formed from a polyester-based adhesion promoter which is at least 30 microns thick applied directly to the said surface (2) provided with the layer (11) of paint.

## Patentansprüche

1. Lackierverfahren, das auf Bauelemente, die aus synthetischen Kunststoffmaterialien gebildet sind, insbesondere auf Bauteile von Kraftfahrzeugen anwendbar ist, die aus Verbundwerkstoffen gebildet sind, **dadurch gekennzeichnet, dass** es die Schritte umfasst:
- Aufbringen einer Schicht (11) eines ersten polymerisierbaren Materials auf eine zu lackierende Oberfläche (2) des besagten Bauelementes (1), wobei das erste polymerisierbare Material von einem Typ ist, der polymerisiert eine Schicht bilden kann, die für eine beliebige gasförmige Substanz undurchlässig ist, und der durch Erwärmen auf eine erste bestimmte Temperatur vollständig polymerisierbar ist,
- Erwärmen des Bauelementes (1) mit der durch die besagte Schicht des ersten polymerisierbaren Materials überdeckten Oberfläche (2), die zu lackieren ist, auf die erste vorbestimmte Temperatur, bis das erste polymerisierbare Material vollständig zur Bildung einer gasundurchlässigen Schicht (11) polymerisiert ist, die die besagte zu lackierende Oberfläche, vollständig überdeckt,
- Aufbringen auf die besagte Oberfläche (2) wenigstens eine Grundschicht (12) mit bestimmter Stärke aus einem polymerisierbaren elektrisch leitenden Material, das durch Erwärmen auf eine zweite vorbestimmte Temperatur polymerisierbar ist,
- Erwärmen des Bauelementes (1) auf die besagte zweite vorbestimmte Temperatur, um eine Polymerisation der besagten Grundschicht (12) aus dem polymerisierbaren elektrisch leitenden Material zu bewirken, so dass die Grundschicht (12) aus dem polymerisierbaren elektrisch leitenden Material nicht direkt auf die zu lackierende Oberfläche (2), sondern auf die gasundurchlässige Schicht (11) aufgebracht ist,
- Aufbringen wenigstens einer Farbschicht (13, 14) oben auf die Grundschicht (12) aus dem elektrisch leitenden polymerisierbaren Material,
wobei das erste polymerisierbare Material so gewählt ist, dass die erste vorbestimmte Temperatur unter sowohl der zweiten vorbestimmten Temperatur als auch der niedrigsten Verdampfungstemperatur der Monomere liegt, die das synthetische Kunststoffmaterial bilden, aus dem das zu lackierende Bauelement besteht.

2. Verfahren nach Anspruch 1, bei dem das zu lackierende Bauelement aus einem Material auf der Basis von in Wärme aushärtenden Vinylester/Polyester-Harzen gebildet ist, **dadurch gekennzeichnet, dass** das zweite polymerisierbare Material aus einer transparenten katalysierten Zweikompontenpolyurethanfarbe besteht.

3. Verfahren nach Anspruch 2, **dadurch gekennzeichnet, dass** das erste polymerisierbare Material oben auf die zu lakkierende Oberfläche (2) so aufgebracht wird, dass darauf eine Schicht mit einer Stärke zwischen 30 und 40 µm gebildet wird.

4. Verfahren nach Anspruch 2 oder Anspruch 3, **dadurch gekennzeichnet, dass** eine Schicht (10) aus einem Haftpromotor für das erste polymerisierbare Material in direktem Kontakt mit der zu lackierenden Oberfläche (2) aufgebracht wird, wobei das erste polymerisierbare Material unmittelbar oben auf die Schicht (10) aufgebracht wird, die aus dem Haftpromotor gebildet ist.

5. Verfahren nach Anspruch 4, **dadurch gekennzeichnet, dass** ein Haftpromotor auf Polyesterbasis ("Barrier") verwandt wird, der auf die zu lackierende Oberfläche (2) in einer durchgehenden Schicht (10) mit einer Stärke von wenigstens 30 µm aufgebracht wird und dass die katalysierten Zweikomponentenpolyurethanfarbe so gewählt wird, dass sie bei einer Temperatur von 60°C vollständig polymerisiert ist.

6. Verfahren nach Anspruch 5, **dadurch gekennzeichnet, dass** die zweite Zweikomponentenpolyurethanfarbe der Oberfläche (2) durch eine Nassverfahren zugeführt wird.

7. Verfahren nach einem der Ansprüche 2 bis 6, **dadurch gekennzeichnet, dass** das elektrisch leitende polymerisierbare Material eine Einkomponentengrundierung ist, die durch Erwärmen auf eine Temperatur von wenigstens 140-150°C polymerisierbar ist.

8. Lackiertes Bauelement (1) aus einem synthetischen Kunstharzmaterial, insbesondere Fahrzeugkarosserieteil aus einem Verbundmaterial mit einer Platte (1), die aus wenigstens einem synthetischen Kunstharzmaterial gepresst ist, dessen wenigstens eine sichtbare Oberfläche (2) mit mehreren Schichten aus polymerisierbaren Materialien überzogen ist, die wenigstens ein Farbschicht (13, 14) einschließen, wobei die Schichten aus polymerisierbaren Materialien in der Reihenfolge beginnend mit der der Oberfläche (2) benachbarten Schicht eine erste gasundurchlässige Schicht (11) und eine zweite gasdurchlässige Schicht (12) umfassen, die beide aus jeweils verschiedenen polymerisierbaren Materialien gebildet sind, wobei das Material, dass die erste Schicht (11) bildet, eine chemische Zusammensetzung derart hat, dass es vollständig beim Erwärmen auf eine erste vorbestimmte Temperatur polymerisiert, das Material, dass die zweite Schicht (12) bildet, eine derartige chemische Zusammensetzung hat, dass es eine elektrisch leitende Grundierung zur Aufnahme der wenigstens einen Farbschicht (13, 14) bildet und polymerisiert, wenn es auf eine zweite vorbestimmte Temperatur erwärmt wird, die im Wesentlichen gleich der Temperatur ist, die zum Polymerisieren der wenigstens einen Farbschicht benötigt wird, welches Bauelement **dadurch gekennzeichnet ist, dass** das Material, das die erste Schicht (11) bildet, so gewählt ist, dass die erste vorbestimmte Temperatur unter sowohl der zweiten vorbestimmten Temperatur als auch der tiefsten Verdampfungstemperatur der Monomere liegt, die das synthetische Kunstharz bilden, aus dem die Platte gebildet ist.

9. Lackiertes Bauelement nach Anspruch 8, **dadurch gekennzeichnet, dass** die Platte (1) aus wenigstens einem in Wärme aushärtenden Harz auf Vinylester/Polyesterbasis gebildet ist und dass die erste Schicht (11) aus einer Zweikomponentenpolyurethanfarbe besteht, wobei die erste Schicht (11) eine Stärke zwischen 30 und 40 µm hat und über eine Schicht (10) aus einem Material aufgebracht ist, die aus einem Haftpromotor auf Polyesterbasis gebildet ist, die eine Stärke von wenigstens 30 µm hat und direkt auf die Oberfläche (2) aufgebracht ist, die mit der Farbschicht (11) versehen ist.

## Revendications

1. Procédé de peinture applicable à des éléments fabriqués en matière plastique synthétique, en particulier des composants de véhicules automobiles fabriqués en matières composites,
**caractérisé en ce qu'**il comprend les étapes de :
application, sur une surface (2) d'un dit élément (1) à peindre, d'une couche (11) d'une première matière polymérisable, la dite première matière polymérisable étant d'un type qui peut former, une fois polymérisée, une couche qui est imperméable à toute substance gazeuse et qui est complètement polymérisable par chauffage à une première température prédéterminée ;
chauffage de l'élément (1), la dite surface (2) à peindre étant couverte avec la dite couche de première matière polymérisable, à la dite première température prédéterminée jusqu'à ce que la dite première matière polymérisable soit complètement polymérisée pour former une couche imperméable aux gaz (11) qui couvre complètement la dite surface à peindre ;
application sur la dite surface (2) d'au moins une couche de base (12) d'une épaisseur prédéterminée d'une matière électriquement conductrice polymérisable, qui est polymérisable par chauffage à une deuxième température prédéterminée ;
chauffage de l'élément (1) à la dite deuxième température pour provoquer la polymérisation de la dite couche de base (12) de matière électriquement conductrice polymérisable, d'une manière telle que la dite couche de base (12) de matière électriquement conductrice polymérisable est déposée indirectement sur la dite surface (2) à peindre mais sur la dite couche imperméable aux gaz (11) ;
application d'au moins une couche de peinture (13, 14) sur le dessus de la dite couche de base (12) de matière polymérisable électriquement conductrice ;
la dite première matière polymérisable étant choisie de sorte que la dite première température prédéterminée soit inférieure à la fois à la dite deuxième température prédéterminée et à la plus basse température de vaporisation des monomères formant la dite matière plastique synthétique qui constitue le dit élément à peindre.

2. Procédé selon la revendication 1, dans lequel le dit élément (1) à peindre est constitué d'une matière à base de résines thermodurcissables de type vinyl ester / polyester, **caractérisé en ce que** la dite deuxième matière polymérisable est constituée d'une peinture transparente catalysée de type polyuréthane à deux composants.

3. Procédé selon la revendication 2, **caractérisé en ce que** la dite première matière polymérisable est appliquée sur le dessus de la dite surface (2) à peindre, pour former sur cette surface une couche (11) d'épaisseur comprise entre 30 µm et 40 µm.

4. Procédé selon la revendication 2 ou la revendication 3, **caractérisé en ce qu'**une couche (10) d'agent favorisant l'adhérence pour la dite première matière polymérisable est appliquée en contact direct avec la dite surface (2) à peindre, cette première matière polymérisable étant appliquée immédiatement sur le dessus de la dite couche (10) formée par l'agent favorisant l'adhérence.

5. Procédé selon la revendication 4, **caractérisé en ce qu'**on utilise un agent favorisant l'adhérence à base de polyester (« Barrière »), appliqué sur la dite surface (2) à peindre en une couche continue (10) d'au moins 30 µm d'épaisseur ; et **en ce que** la dite peinture catalysée de type polyuréthane à deux composants est choisie de sorte qu'elle est complètement polymérisée à une température de 60°C.

6. Procédé selon la revendication 5, **caractérisé en ce que** la dite deuxième peinture de type polyuréthane à deux composants est appliquée sur la dite surface (2) par une technique « humide sur humide ».

7. Procédé selon une quelconque des revendications 2 à 6, **caractérisé en ce que** la dite matière polymérisable électriquement conductrice est un apprêt à composant unique qui est polymérisable par chauffage à une température d'au moins 140 à 150°C.

8. Elément peint (1) formé à partir d'une matière plastique synthétique, en particulier un élément de carrosserie de véhicule formé à partir d'une matière composite, comprenant un panneau (1) pressé à partir d'au moins une résine plastique synthétique dont au moins une surface visible (2) est couverte par une pluralité de couches de matières polymérisables incluant au moins une couche de peinture (13, 14) ; la dite pluralité de couches de matières polymérisables comprenant, dans l'ordre en partant de la couche adjacente à la dite surface (2), une première couche imperméable aux gaz (11) et une deuxième couche perméable aux gaz (12), toutes deux formées en matières polymérisées différentes ; la matière formant la première couche (11) ayant une composition chimique telle qu'elle polymérise complètement par chauffage à une première température prédéterminée ; la matière formant la deuxième couche (12) ayant une composition chimique telle qu'elle forme un apprêt électriquement conducteur pour recevoir la dite au moins une couche de peinture (13, 14) et qu'elle polymérise par chauffage à une deuxième température prédéterminée qui est sensiblement égale à celle qui est nécessaire pour polymériser la dite au moins une couche de peinture ;
l'élément étant **caractérisé en ce que** la matière formant la première couche (11) a été choisie d'une manière telle que la dite première température prédéterminée est inférieure à la fois à la dite deuxième température prédéterminée et à la plus basse température de vaporisation des monomères formant la dite résine plastique synthétique à partir de laquelle le dit panneau est fabriqué.

9. Elément peint selon la revendication 8, **caractérisé en ce que** le dit panneau (1) est formé à partir d'au moins une résine thermodurcissable à base de vinyl ester / polyester , et **en ce que** la première couche (11) est formée d'une peinture de type polyuréthane à deux composants, la dite première couche (11) ayant une épaisseur comprise entre 30 et 40 µm et étant appliquée sur une couche (10) d'une matière formée d'un agent favorisant l'adhérence à base de polyester qui a une épaisseur d'au moins 30 µm, appliquée directement sur la dite surface (2) et portant la couche (11) de peinture.
